

May 14, 1940.

C. J. KOEBEL

2,200,281

ART OF SETTING DIAMONDS FOR INDUSTRIAL PURPOSES

Filed July 28, 1937

2 Sheets-Sheet 1



INVENTOR  
Charles J. Koebel  
BY  
J. E. Decker  
ATTORNEY

May 14, 1940.

C. J. KOEBEL

2,200,281

ART OF SETTING DIAMONDS FOR INDUSTRIAL PURPOSES

Filed July 28, 1937

2 Sheets-Sheet 2

*Fig. 18*



*Fig. 19*



INVENTOR  
*Charles J. Koebel*  
BY  
*Velv Peeler*  
ATTORNEY

## UNITED STATES PATENT OFFICE

2,200,281

ART OF SETTING DIAMONDS FOR  
INDUSTRIAL PURPOSES

Charles J. Koebel, Detroit, Mich.

Application July 28, 1937, Serial No. 156,223

9 Claims. (Cl. 76—108)

Diamond-carrying tools that are now so increasingly used in the industrial arts are subject to great stress and strain. The setting or mounting which carries the diamond must therefore hold it with great firmness and must be capable of resisting the heat generated by the cutting action of the tool against the work acted upon. Diamonds, when being set, cannot be subjected to excessive temperatures as that tends to destroy the valuable properties of the stones, and therefore processes that involve the production of a setting by casting molten metal around the stone have not been successful to any great extent. It has also been attempted to produce a hardened slug and thereafter to set the diamond in the slug as by peening the metal over the stone, but this necessarily means that the labor of peening the hard metal of the setting is very difficult and slow and requires highly skillful working. Moreover, to obtain a sufficiently strong setting, the stone must have a fairly pronounced girdle or equator so that the metal may be worked over it to adequately grip the stone and prevent it from coming loose, and this renders many relatively inexpensive diamonds, that would otherwise be suitable for the purpose, unfit for use on account of their shape. There is still another disadvantage in peening hard metal over a stone, and that is a tendency to break the stone during the process of peening. It has been attempted to overcome this by drilling a relatively large hole or otherwise forming an aperture in a metal slug and filling the hole around the diamond with a brazing material, but this too has been found unsuitable in that the setting is not strong enough and, in the case of a corebit carrying numerous diamonds, it, as well as the peening process, requires each diamond to be set individually—necessarily a slow method. In Patent No. 1,848,182 of March 8, 1932, is disclosed an invention in which a diamond is imbedded in a body of comminuted metallic material, and thereafter sintered. This process has been extensively used and is in successful operation today but when the comminuted material is subjected to pressure the diamond, if its longest dimension extends in the direction in which pressure is exerted when compressing the comminuted material before sintering, will naturally tend to change its position in the material and this is objectionable because the pointed end of such diamond is more effective as a cutting surface than the more blunt portion. To overcome this, the use of diamonds that are relatively longer in one direction than in the other is avoided, and this again constitutes

a limitation upon the character of the stones that are usable.

The main object and feature of this invention is to overcome these various disadvantages, and to provide a method whereby inexpensive material can be successfully used to set diamonds of practically any shape and which requires in practice very little expert skill and one which, while admitting of the individual seating or positioning of a plurality of diamonds on a readily workable carrying member, permits simultaneous setting of the individually seated stones; and also in which the step of hardening the setting is carried on after the diamonds have been individually positioned and at temperatures well below the critical point at which the character of the stone becomes adversely affected.

In the accompanying drawings several preferred exemplifications of the invention are disclosed, and in said drawings:

Fig. 1 is a vertical sectional view of one form of mold for compressing comminuted metallic material;

Fig. 2 is a diagrammatic representation of one form of sintering furnace that may be used in connection with the invention;

Figs. 3 and 4 are respectively edge and plan views of one form of carrying member that may be used in carrying out the invention;

Figs. 5 and 6 are views similar to Figs. 3 and 4 but showing diamonds preliminarily positioned or seated on the carrying member;

Fig. 7 is a fragmentary detail sectional view of a portion of a carrying member with two methods of seating the diamonds indicated;

Fig. 8 is a view similar to Fig. 1 but showing the compressing of an additional body of comminuted material around the stones that have been seated in the carrying member;

Fig. 9 shows the placing of a body of copper on the comminuted material and the assemblage laced in a suitable mold for sintering the additional body of comminuted material and hardening the setting;

Figs. 10 and 11 are views similar to Figs. 5 and 6, but show the finished product;

Figs. 12 and 13 are respectively edge and plan views of a different form of carrying member;

Figs. 14 and 15 are views similar to Figs. 12 and 13 but show a coating of paste of comminuted metallic material and diamond particles applied to the carrying member;

Fig. 16 is a view similar to Fig. 14 but shows a body of copper placed on top of the assemblage of Fig. 14;

20

25

30

35

40

45

50

55

Fig. 17 is a view similar to Fig. 16 but shows the finished product;

Fig. 18 is a top plan view of a muffle that may be employed in place of the mold shown in Fig. 9 for the sintering operation; and

Fig. 19 is a section on the line 19, 19 of Fig. 18.

In carrying out the process of my invention I first produce a carrying member that is, with respect to the final hardness of setting desired, relatively soft. The material used can be principally iron, and I have found Swedish iron with a slight admixture of cobalt and copper to be a suitable medium. As an exemplification of the material that can be used the following formula is given:

|              | Per cent |
|--------------|----------|
| Swedish iron | 89       |
| Cobalt       | 6        |
| 20 Copper    | 5        |
|              | 100      |

Preferably the metallic material is comminuted or reduced to powder form of say three hundred and twenty five mesh and thoroughly mixed as by ball milling for one hour. A body of powder 25 is then placed in a mold as 26 provided with a bottom molding die 26' and subjected to a pressure of from twenty to thirty tons by means of a plunger 27 to compress the material into a fairly stable body. As the shape of the carrying member to be produced here happens to be ring-like, a center post 28 is carried by the mold to produce the circular opening in the carrying member. The member thus produced, indicated by 29, is then placed in a sintering furnace 30 of any suitable construction and from which air is excluded where it is sintered at a temperature of say 1200° centigrade. One form of furnace that may be employed for this purpose is disclosed in my Patent No. 1,848,182 of March 8, 1932. Carrying member 29 thus produced has shrunk but slightly, about one percent or less, and is readily workable in that it has a hardness of from forty-five to fifty-one according to Rockwell hardness testing device. According to the procedure illustrated in Fig. 1, the carrying member is pressed with a radius prior to the sintering treatment but if desired, said carrying member 50 may be pressed in some rectilinear form and a radius turned thereon after the sintering treatment. After the carrying member is cooled to room temperature, one or more diamonds or diamond particles are preliminarily positioned or seated on said member. Fig. 7 exemplifies this operation, and it will be seen that apertures as 31 and 32 can be readily formed in the carrying member as by drilling and it will be noted that the size and shape of these apertures can be different so as to suit the size and shape of different stones as 33 and 34. To hold the stone temporarily in position it may be lightly tapped as indicated in connection with 33, the lower end 35 of which is slightly imbedded in the relatively soft material of the carrying member or, as indicated in connection with 34, the relatively soft metal can be peened over as at 36 to retain the stone in position. The particular tool here selected to illustrate the invention is a corebit 55 and, as shown in Figs. 5 and 6, a number of diamonds will be seated on the carrying member in such relative position as will render the tool most effective. The surface or surfaces that carry the stones are now covered with a body of comminuted material 37 of the same character as

that used in forming the carrying member. This body of comminuted material may be either in powder or paste form and, if in powder form, it may be slightly compressed to fill the interstices around the stones, as by placing it in a suitable mold as 38 and subjecting it to the action of a plunger 39 that may be operated by hand. If it is desired to use the material in paste form, a slight amount of paraffin can be added thereto, and the paste smeared and packed around and over the stones. A body of copper 40 or other material, as silver solder, having a lower melting point than the comminuted material is now placed on the body of comminuted material 37 and the assemblage thus produced is sintered at a temperature slightly below that used in sintering the original carrying member. I have found a temperature of 1174° centigrade suitable for this purpose. The result of this action is that the individually positioned stones are set simultaneously and permanently by the creation of a sintered extension on the original carrying member. At the same time, the body of copper or other material insinuates itself through the carrying member and hardens the setting to about ninety-seven or eight according to the Rockwell hardness testing device. The copper used will preferably be electrolytic copper and I have found a body of copper equal to forty percent by weight of the material used to produce the original carrying member gives good results. I have found that the amount of copper needed depends upon the pressure to which the comminuted material of the carrying member is subjected. The more highly compressed the comminuted material is, the less copper is needed. The sintering can conveniently be carried on in a carbon mold 41 or a graphite boat 46, or other suitable device for the purpose, that can be placed in a furnace like 30. According to the arrangement shown in Figs. 18 and 19, diamond-studded slug 29 is placed upon slabs 47 of alundum in boat 46 after comminuted metal 48 in powdered or paste form has been applied to the diamond-studded surfaces and surmounted by a body 49 of copper or other suitable material, as described above, the complete assemblage being placed in sintering furnace 30. It will be noted that the steps are carried on at temperatures well below the critical temperature, about 1380° centigrade at which the desirable qualities of the diamonds are adversely affected. The finished product is indicated at 42 in Figs. 10 and 11 and will usually require some sandblasting to properly expose the diamonds. The ring-like member thus produced is then mounted in any suitable manner on a holder, as by brazing, welding or otherwise.

A modification of the above process is as follows. The comminuted metal previously described is compressed under a pressure of from twenty to thirty tons and heated in furnace 38 at a temperature of 950° centigrade, thereby producing a carrying member having a hardness of only eleven with respect to the Rockwell hardness testing device. The holes are then drilled and the diamonds preliminarily positioned and a body of comminuted metal of the same character as that used in producing the carrying member is applied over and around the stones, but no body of copper is applied at this point. The body of comminuted metal is then subjected to a pressure of thirty tons and sintered in a furnace such as 30 at a temperature of 1175° centigrade, thereby setting the diamonds and increasing the hard- 75

ness of the carrying member to fifty-five according to the Rockwell hardness testing device. After cooling the setting, a body of copper is then applied to the surface carrying the diamonds and the assemblage is heated to a temperature of 1174° centigrade, thereby obtaining a hardness of ninety-four or five according to the Rockwell hardness testing device. The advantage of this mode of operation is that there is practically no shrinkage of the setting after it has been sintered at a temperature of 1175° centigrade.

It will, of course, be understood that the invention is not limited to the production of core-bits or that, if used for the production of core-bits, it is necessary to produce a ring-like setting. The diamonds can be set in slugs and the slugs mounted in slots or otherwise on a holder as shown, for instance, in my application Ser. No. 121,935, filed January 23, 1937.

In Figs. 12 to 17 is illustrated an abrasive tool in which diamond particles instead of relatively large diamonds are used. In this case a carrying member 43, here in the form of a disk, of relatively soft material is produced as before. A mixture 44 of diamond particles and comminuted metal of the character previously described and having a small amount of paraffin is then applied to the surface of the disk as indicated in Fig. 14. The assemblage is then subjected to pressure thereby positioning the diamond particles in the soft carrying member. A body of copper 45 is then placed on the surface carrying the diamond particles and the assemblage is then sintered at a temperature slightly below that initially used in sintering the carrying member. It will be understood that one or more or all of the surfaces of the carrying member may be provided with the abrasive mixture described.

I claim:

1. The method of setting a diamond for industrial purposes which consists in: sintering a compressed body of comminuted metallic material composed principally of iron having a slight admixture of cobalt and copper to form a relatively soft porous carrying member; preliminarily positioning a diamond on the carrying member thus produced; applying to that surface of the carrying member on which the diamond is carried a layer of comminuted metallic material of substantially the same character as that originally used in producing the carrying member; applying a body of copper to the surface of the layer of comminuted material; and subjecting the assemblage to heat at a temperature lower than that used in sintering the carrying member but sufficiently high to sinter the layer of comminuted metallic material and to cause the copper to insinuate itself into the carrying member to thereby harden the latter and set the diamond permanently.

2. The method of setting a diamond for industrial purposes which consists in: sintering a compressed body of comminuted metallic material composed principally of iron to form a relatively soft carrying member; forming an aperture in said carrying member; seating a diamond in said aperture; applying to that surface of the carrying member on which the diamond is carried a layer of comminuted metallic material; compressing said layer of material and subjecting it to a temperature above that used in producing the carrying member but below the point at which the desirable qualities of the diamond are adversely affected; applying a body of copper to the

surface carrying the diamond and subjecting it to a temperature above that used in originally producing the carrying member but below that used in heating the layer of comminuted material.

3. The method of making an abrasive tool which consists in producing a relatively soft porous metallic carrying member by sintering a body of compressed comminuted metallic material, coating one or more surfaces of said member with a mixture of comminuted metallic material and diamond particles, applying to said coating a body of metallic material having a lower melting point than that of said coating, and then subjecting the assemblage to heat at a temperature below that used in originally sintering the carrying member but sufficiently high to sinter the comminuted metallic material and to cause the body of metallic material to insinuate itself into the carrying member.

4. The method of making an abrasive tool which consists in producing a relatively rigid but relatively soft porous metallic carrying member consisting principally of iron by sintering a body of compressed comminuted metallic material, coating one or more surfaces of said member with a mixture of diamond particles and comminuted metallic material, principally iron, applying a body of copper to said coating and then subjecting the assemblage to heat at a temperature below that used in originally sintering the carrying member but sufficiently high to sinter the comminuted metallic material and to cause the copper to insinuate itself into the carrying member.

5. The method of setting a diamond for industrial purposes which consists in: producing a relatively soft and porous metallic carrying member by sintering a body of comminuted metallic material; preliminarily positioning a diamond on said carrying member in a layer of comminuted metallic material; applying to said layer a body of metallic material having a lower melting point than that of said layer; and then subjecting the assemblage to heat at a temperature below that used in originally sintering the carrying member but sufficiently high to sinter the layer and to cause the metal having the lower melting point to insinuate itself into the carrying member, to thereby set the diamond permanently and harden the carrying member.

6. The method of setting a diamond for industrial purposes which consists in: producing a relatively soft and porous metallic carrying member by sintering a body of comminuted metallic material; preliminarily positioning a diamond on said carrying member in a layer of comminuted metallic material of substantially the same character as that originally used in producing the carrying member; applying to said layer a body of metallic material having a lower melting point than that of said layer; and then subjecting the assemblage to heat at a temperature below that used in originally sintering the carrying member but sufficiently high to sinter the layer and to cause the metal having the lower melting point to insinuate itself into the carrying member, to thereby set the diamond permanently and harden the carrying member.

7. The method of setting a diamond for industrial purposes which consists in: producing a relatively soft and porous metallic carrying member by sintering a body of comminuted metallic material composed principally of iron; preliminarily positioning a diamond on said carrying

member in a layer of comminuted metallic material; applying to said layer a body of metallic material having a lower melting point than that of said layer; and then subjecting the assemblage to heat at a temperature below that used in originally sintering the carrying member but sufficiently high to sinter the layer and to cause the metal having the lower melting point to insinuate itself into the carrying member, to thereby set the diamond permanently and harden the carrying member.

8. The method of setting a diamond for industrial purposes which consists in: producing a relatively soft and porous metallic carrying member by sintering a body of comminuted metallic material composed principally of iron; preliminarily positioning a diamond on said carrying member in a layer of comminuted metallic material of substantially the same character as that originally used in producing the carrying member; applying to said layer a body of metallic material having a lower melting point than that of said layer; and then subjecting the assemblage to heat at a temperature below that used in originally sintering the carrying member but

sufficiently high to sinter the layer and to cause the metal having the lower melting point to insinuate itself into the carrying member, to thereby set the diamond permanently and harden the carrying member.

9. The method of setting a diamond for industrial purposes which consists in: sintering a compressed body of comminuted metallic material to form a relatively soft porous carrying member; forming an aperture in said carrying member; seating a diamond in said aperture; applying to that surface of the carrying member on which the diamond is carried a layer of comminuted metallic material; compressing said layer of material and subjecting it to a temperature above that used in producing the carrying member but below the point at which the desirable qualities of the diamond are adversely affected; applying a body of material having a lower melting point than that of said layer to the surface carrying the diamond and subjecting it to a temperature above that used in originally producing the carrying member but below that used in heating the layer of comminuted material.

CHARLES J. KOEBEL. 25